

# UNITED STATES PATENT OFFICE.

HORACE VAUGHN, OF PROVIDENCE, RHODE ISLAND.

## IMPROVEMENT IN COMPOSITIONS FOR WORKING STEEL.

Specification forming part of Letters Patent No. 15,161, dated June 17, 1856.

*To all whom it may concern:*

Be it known that I, HORACE VAUGHN, of the city and county of Providence, and State of Rhode Island, have invented a new and Improved Method of Hardening and Tempering Steel; and I do hereby declare the following to be a full, clear, and exact description of the same.

In order to enable others to use my invention, I will first state the effect of my process and composition upon steel, and then describe the nature of the composition and its mode of application.

First. You both harden and temper at the same time, whereas by the ordinary process the steel is first hardened and then the hard drawn out to a proper temper.

Second. The time required by this system is about one-fourth of that of the old.

Third. It leaves a smooth surface and does not scale.

Fourth. It does not crack, split, warp, or spring after being thus prepared.

Fifth. The more it is heated and hardened the finer and stronger it grows, and this effect is just the reverse of that by the old method.

Sixth. Cast-iron is effectually hardened in such parts as are the more subject to friction or wear.

I will now describe the nature of the composition, and then of the method of applying the same in order to effect the desired object.

There are several known compositions of chemical matter which have been used from time to time in hopes of effecting these results, and none of them have as yet been more than partially successful. Chemical solutions or materials in a liquid state have been the agents often adopted. Solids have been and are now in common use—such as borax, prussiate of potash, &c.—and these, as well as the fluids, are applied at various and generally high stages of heat. The materials mentioned as “solids” and now in use fall far behind the composition or mixed ingredients used by me, as do the fluids behind them, since the volatile part of the latter are so speedily evaporated by the heat as to leave their effect, when applied to heated steel, but trifling. The mixture, however, of the bichromate and prussiate of potash with chloride of sodium in certain proportions will

effect every and all the results we have claimed as the advantages of this over the ordinary system of hardening and tempering, and this is done at comparatively low stages of heat when compared with the old method. This composition is used in a dry pulverized (finely) state and in about the following proportions, viz: two ounces of bichromate of potash, fourteen ounces of prussiate of potash, and seventeen ounces of chloride of sodium. These numbers are not imperative, but are found as good as any in practice; or the chloride of sodium may be used with either the bichromate or the prussiate of potash or articles possessing similar chemical properties as these latter, but in this case the proportion of either of the latter to the chloride of sodium would be about as sixteen to seventeen. The work to be done (the kind of work) would, however, regulate these proportions in a great measure.

Having fully explained the compound, I will only add that it must be finely pulverized, put in a common dredging-box, and from this shaken upon the metal when of proper temperature to receive it. In order to clearly understand when the metal is thus ready it will be necessary to speak in detail of the manner of dealing with a few articles, classified according to the requisite degree of heat.

Dies for heading screws, dies for transferring from steel to or upon steel, and trip-hammer dies, &c., will be considered as the first class for illustration. Heat the steel so that if wood is drawn across it sparks will be freely thrown out. Then sift the composition evenly and freely upon it. Return the steel to a slow and even fire until it is nearly or quite cherry red, and if an exceeding hard and deep temper is required apply the composition a second time at cherry heat, and almost immediately plunge it into cold water.

For the second class—such as fluted reamers, cutters, and large taps—harden by a shade less in degree of heat than cherry red, and sprinkle with the composition but once, then plunge into cold water.

For the third class—such as small taps and drills for drilling iron—a less degree of heat than the last, sprinkle with composition, and soon plunge into cold water.

Fourth class—such as chisels, gages, and

delicate dies—heat at a lower degree than the last, (or of a dark blood-red heat,) and put on the composition, and as a general rule the composition must be put on when the metal is sufficiently heated to melt it quickly.

These matters have been arranged thus in classes the better to point out and simplify an operation or process as varied as the number of articles upon which we are required to act, and it is done more especially for the purpose of systematizing a very complex operation, except when considered in detail.

What I claim as my invention, and desire to secure by Letters Patent, is—

The dry compound of chloride of sodium and bichromate of potash, with or without the prussiate of potash, for hardening and tempering steel, combined, applied, and operating substantially as is herein set forth.

HORACE VAUGHN.

In presence of—

RHEMIAH KEEN,  
GEO. C. THOMAS.